

J. G. A. RHODIN,  
METHOD OF UTILIZING FELDSPAR,  
APPLICATION FILED DEC. 4, 1915.

1,232,977.

Patented July 10, 1917.



Fig. 1.



Fig. 2.

John Gustaf Adolf Rhodin  
By B. Smigaj  
Atty

# UNITED STATES PATENT OFFICE.

JOHN GUSTAF ADOLF RHODIN, OF CHISWICK, ENGLAND.

## METHOD OF UTILIZING FELDSPAR.

1,232,977.

Specification of Letters Patent. Patented July 10, 1917.

Application filed December 4, 1915. Serial No. 65,065.

To all whom it may concern:

Be it known that I, JOHN GUSTAF ADOLF RHODIN, residing at 43 Alwyn avenue, Chiswick, Middlesex, England, have invented certain new and useful Improvements in the Method of Utilizing Feldspar and I do hereby declare the following to be a full, clear, and exact description of the invention, such as will enable others skilled in the art to which it appertains to make and use the same.

This invention relates to an improved process for the utilization of potash feldspar (orthoclase).

Orthoclase is a potassium aluminium silicate of fairly constant composition. For a long time it was supposed to be very difficult to decompose, but it has recently been found that decomposition can be effected in various ways by means of alkaline, acid, or indifferent reagents. Fine sub-division of the mineral and the temperature conditions under which the reaction takes place have been found to be of the greatest importance. I have previously described how the potassium contents in orthoclase can be obtained with a very satisfactory yield, but these earlier processes involved the addition of considerable quantities of lime and common salt, and the potassium was eventually obtained in the form of chlorid. It is, however, frequently preferable to obtain the sulfate, and one of the objects of the present invention is the production from orthoclase of potassium sulfate, but other objects will become apparent in the course of the present specification.

It is already well known that sulfate of potash can be obtained by the action of sulfuric acid upon orthoclase, and that the yield will increase with the fineness of the mineral powder, but this yield is by no means a complete one. It is also known that if an atmosphere of damp sulfurous acid is allowed to act upon feldspar at room temperatures and in closed vessels decomposition takes place and a certain amount of sulfates are obtained, but neither of these reactions are suited for a manufacturing process, and a further object of the present invention is consequently to increase the yield of potassium sulfate per time unit and unit of plant. I have discovered that this end may be achieved by using a contact process for the manufacture of sulfuric acid in which the contact substance is finely di-

vided feldspar together with certain additions to be described over which sulfurous acid, steam, and air are passed at a temperature exceeding but not greatly exceeding the boiling point of sulfuric acid. Under these circumstances the reaction is very energetic, and the sulfuric acid actually forms on the mineral powder, while an excess of gas mixture leads to the formation of strong sulfuric acid which does not condense in the mineral but which can be recovered in suitable apparatus and used for commercial purposes. If desired the formation of the strong acid can usually be avoided by carefully regulating the quantities of the reagents according to well known practice. As additions to the powdered feldspar, I may use the chlorids or nitrates of sodium, magnesium, calcium, or similar metals, and in quantities not exceeding two per cent. of the weight of the spar, although very much smaller quantities will usually be found effective. When the decomposition has approached or reached completion the charge is drawn and the potassium sulfate is washed out with water and obtained by crystallization leaving a silicate residue which may be used for various purposes. I prefer to use it for the manufacture of white Portland or Roman cement in a manner to be described. It will thus be seen that my present invention provides a complete process for the utilization of potash feldspar and for the manufacture therefrom of sulfate of potash as well as of by-products of great commercial value.

The invention is carried out as follows, and is illustrated in the accompanying drawings in which Figure 1 shows a section of a suitable apparatus for carrying out the invention, while Fig. 2 is a plan view. The complete plant necessary for carrying out this invention is more or less complicated, but is well known in sulfuric acid technology, and the drawings are given as a schematic design of the furnace part of the plant, although it will be understood that condensing apparatus, washing and crystallizing plant for the sulfate of potash, and other well known integers of plant or machinery in which no novelty *per se* resides will be required.

The feldspar is to begin with ground very fine in a quartzite lined tube mill preferably charged with pebbles, although a preliminary crushing in a ball mill may some-

times be necessary. The ground material should leave practically no residue on a 180 mesh standard cement sieve. Accelerating salt, *e. g.* common salt or sodium chlorid 5 is preferably added by impregnating the feldspar powder with a solution of the salt. In most cases half per cent. by weight is added to the feldspar with just enough water to make the whole mass damp, although, 10 as previously stated, the amount of salt will in no case have to exceed two per cent. The mass is then charged into a simple tubular retort A of impervious acid-proof earthenware, having at one end a charging and 15 discharging door B. The retort is mounted in a furnace C of the reverberatory type. At the rear or charging and discharging end, inlet tubes D are provided for the gas mixture, while at the other end of the retort at E a suitable connection is made with 20 condensing plant F.

In operation a charge G of salt impregnated spar is put into the retort which is kept at very dull red heat for a suitable 25 time, while a mixture of sulfurous acid, steam, and air is passed over the charge. The time of reaction varies with several factors such as the actual composition of the gas mixture, the temperature, and the fineness 30 of division of the mineral. With regard to the composition of the gas mixture, this will carry more or less nitrogen according to the working of the pyrites or brimstone burners which will obviously be necessary. For this reason it would be preferable 35 to work with pure sulfur di-oxid, but for economic reasons this will seldom be practicable. Further, the feldspar itself varies in different localities, and the orthoclase 40 is in many places impregnated with various forms of soda spar. It should be pointed out that the more closely the chemical composition of the spar approaches that of pure orthoclase, the more suited the mineral will 45 be for the purposes of this invention. The gas mixture is made and adjusted in any of the well known types of plant used for the contact process of sulfuric acid manufacture.

50 In some cases it may be necessary to stoke up the furnace and raise the tempera-

ture to complete the reaction, but by suitably adjusting all factors the time for the decomposing of a thin layer of powdered spar should not exceed one hour. The gases 55 are then turned off and the charge is drawn, the furnace being of course re-started with a new charge immediately.

The drawn charge is lixiviated with water and the potassium sulfate is recovered by 60 evaporation.

The white acid aluminum silicate residue is made into cement slurry with the addition either of dry slaked lime or ground limestone, neither of which should contain any 65 coloring oxids. The proportions depend upon whether it is desired to make a Roman or a Portland cement. For whiteness a Roman cement containing fifty per cent. of CaO is preferable, but an addition of two- 70 and-a-half per cent. of alum or of a corresponding quantity of lime cake is essential.

A Portland cement may be made in the usual way, clinkered and ground, but it will always retain a greenish tint. 75

I claim:—

1. The method of utilizing potash feldspar which consists in mixing the ground feldspar with a small quantity of a sodium salt, causing a mixture of sulfur dioxid, 80 steam and air to react on the heated mixture, collecting the sulfuric acid formed in suitable receivers and leaching the residue so as to obtain sulfate of potash and to leave a residue suitable for making white Roman 85 or Portland cement.

2. The method of utilizing potash feldspar which consists in mixing the ground feldspar with a small quantity of sodium chlorid, causing a mixture of sulfur dioxid, 90 steam and air to react on the heated mixture collecting the sulfuric acid formed in suitable receivers and leaching the residue so as to obtain sulfate of potash, and to leave a residue suitable for making white Roman 95 or Portland cement.

In testimony whereof I affix my signature in presence of two witnesses.

JOHN GUSTAF ADOLF RHODIN.

Witnesses:

FRANK B. DEHN,  
ALBERT R. RAMSEY.